

March 8, 1927.

1,620,511

E. R. BERRY

QUARTZ WORKING

Filed April 18, 1923

2 Sheets-Sheet 1

Fig. 1.



Inventor  
Edward R. Berry  
By Alexander S. Lutz  
His Attorney

March 8, 1927.

1,620,511

E. R. BERRY

QUARTZ WORKING

Filed April 18, 1923

2 Sheets-Sheet 2

Fig. 2.



Inventor  
Edward R. Berry  
By Alexander S. Lunt  
His Attorney.

## UNITED STATES PATENT OFFICE.

EDWARD R. BERRY, OF MALDEN, MASSACHUSETTS, ASSIGNOR TO GENERAL ELECTRIC COMPANY, A CORPORATION OF NEW YORK.

## QUARTZ WORKING.

Application filed April 18, 1923. Serial No. 633,017.

The present invention relates to the manufacture of elongated objects, such as rods or tubes, from fused or amorphous quartz. It is the object of my invention to improve 5 the uniformity of the process, to render the process more convenient, and to reduce the supervision required.

Formerly plastic quartz cane or tube when issuing from an extrusion apparatus has 10 been caused to enter a body of water which cooled and thereby set or hardened the cane. As the water only partially counterbalanced the weight of the cane or tube, the plastic cane or tube became reduced in diameter at the extrusion orifice, as the extrusion 15 progressed and the tractive force exerted by the extruded cane became appreciable.

In accordance with my present invention the weight of the extruded quartz is counterbalanced either by a liquid of approximately 20 the same specific gravity as quartz; or wholly or partly by mechanical means.

Fig. 1 illustrates my invention as carried out with a liquid of higher specific gravity 25 than water and Fig. 2 illustrates the same as applied to a mechanical counterbalance.

In Fig. 1 the furnace from which the plastic cane is extruded is indicated only, most of the furnace being broken away, as 30 it constitutes no part of my invention. The drawing shows the supporting platform 2 upon which rests the base 3 of the furnace. The heater tube 4 makes contact with a water-cooled terminal 5 to which are connected current supply conductors 6, 7. The quartz cane 8 issuing from the heated zone 35 of the furnace (for example, through an orifice not shown) is projected into a body of liquid 9 contained in a tubular receptacle 40 10. The liquid should have a specific gravity of about 1.5 to 2.2 or even higher in some cases where large rods of about 1"

diameter are being made, and may consist of a solution of a salt, such as mercuric potassium iodide or of a solution of a heavy liquid 45 such as sulphuric acid. Liquid organic compounds, such for example as carbon tetrachloride, also may be used. The liquid column has been indicated as broken as it may be of greater length than otherwise 50 could be indicated in the drawing. The resulting strip 8 is of uniform diameter.

As shown in Fig. 2, the strip 8 may be mechanically counterbalanced by a platform 11 carried by an endless belt 12, running 55 over pulleys 13, 14. When the platform 11 descends the belt picks up a flexible weight or chain 15 so as to give a gradually increasing upward thrust to counterbalance the progressively increasing weight of the 60 cane 8 in order to reduce traction upon the still plastic material issuing from the extrusion apparatus.

The drawing shows the pulleys and belt operating in a body of water or other liquid 65 16, but this liquid may be omitted and the descending quartz cane 8 may be cooled by a current of air. The cooling liquid in the tank 10 of either modification may be drawn off by a discharge duct 17.

Although I have described my invention with reference to the manufacture of quartz cane, I wish it to be understood that tubing or other elongated objects may be made in the same manner.

What I claim as new and desire to secure by Letters Patent of the United States, is:—  
The process of shaping plastic silica which consists in projecting the same in an elongated form into a liquid having approximately the same specific gravity as silica.

In witness whereof, I have hereunto set my hand this 14th day of April, 1923.

EDWARD R. BERRY.